

June 18, 1940.

F. C. ATWOOD

2,204,746

PACKAGE AND NONCORRODIBLE CONTAINER

Filed Sept. 24, 1936



INVENTOR

BY Francis Clark Atwood  
J. Stanley Churchill  
ATTORNEY.

## UNITED STATES PATENT OFFICE

2,204,746

## PACKAGE AND NONCORRODIBLE CONTAINER

Francis Clarke Atwood, Newton, Mass., assignor to Atlantic Research Associates, Inc., a corporation of Delaware

Application September 24, 1936, Serial No. 102,360

1 Claim. (Cl. 220--64)

This invention relates to a novel package and noncorrodible container.

One object of the present invention is to provide a novel package containing protein material and water and which is adapted to enable the protein material to be kept for long periods of time without corrosion of the container and the accompanying contamination of the protein material as a result of the solution of portions of the container.

Another object of the invention is to provide a novel and highly useful noncorrodible container which is particularly adapted among other uses for holding materials of a protein nature which at the present time present difficulties as a result of the corrosive action of such materials in the presence of water upon the inner portions of the metal cans which have heretofore been used.

With these general objects in view, and such others as may hereinafter appear, the invention consists in the package and in the noncorrodible container used in producing the package herein-after described and particularly defined in the claim at the end of this specification.

25 The drawing illustrates in vertical section the present package and noncorrodible container.

The problem of packaging corrodible materials, and particularly those embodying water in metal containers has proven difficult of solution. For example, in the packaging of materials of a protein nature such as glues, casein paints, and various other water paints, metal pails and cans have been employed but difficulty has been experienced in protecting the inner surfaces of the can or pail from the corrosive effect of the water solution or emulsion of such protein materials. In the presence of water the protein materials are acidic in nature and accelerate corrosion of the steel, tin plate, or other materials which have heretofore been commercially used in the attempt to protect the inside of the metal containers. Attempts have also been made to utilize lacquers but such lacquer coatings gradually soften under the continuous exposure to water for relatively long periods of time, with the result that corrosion of the containers has occurred and has contaminated the water paint or other material with the products resulting from the corrosion.

Referring now to the drawing, 10 represents a container, preferably of metal, and which is provided upon its inner surface with a protective film 12 of wool fat. It is preferred to utilize lanolin or commercial forms of purified wool wax, wool grease or degras. In producing the

present package the water mixture or solution as the case may be of the corrodible material to be packaged and which preferably may comprise a protein material such as glue, casein, and the like, is contained within the prepared container, 5 and as herein illustrated such material is indicated at 13. The container may be provided with a cover member 14, the under surface of which may also be provided with the protective film 12 of the lanolin, wool grease, wool wax, or 10 degras.

In the application of the film 12 to the inner surfaces of the container 10 and cover member 14, I prefer to utilize anhydrous lanolin, wool wax, or degras, and render the same fluid with 15 turpentine or solvent spirits of any suitable nature after which the film may be applied by brushing or otherwise.

The present container has been found to be capable of storing the corrodible protein material 20 for long periods of time with no effect upon the container and with the elimination of the contamination of the material as a result of corrosive action.

While the present container with its improved 25 protective film lends itself particularly to the production of a noncorrodible package embodying a corrodible protein material, nevertheless it will be understood that the container may be used with advantage for the reception and storage of 30 other materials which possess corrosive action upon metal containers.

In describing and claiming my invention I use the term "wool fat" as a generic term for the class of coating materials disclosed, namely, lanolin, wool wax, wool grease or degras.

Having thus described the invention, what is claimed is:

A package comprising a metal container, a cover member therefor for closing the container, both the cover member and the container being formed from a metal that is corroded by an aqueous casein paint, said cover and container being provided with a protective film of wool fat at all portions where said paint would normally 40 contact said metal, and an aqueous casein paint within said container which is separated from said metal by said protective film of wool fat, whereby the metal is protected from corrosion due to the paint, and the paint may be stirred 45 in the container without objectionable contamination by the wool fat.

FRANCIS CLARKE ATWOOD.